

## UNITED STATES PATENT OFFICE

2,469,737

## ADDITION AGENT FOR GASOLINE

John G. McNab, Cranford, and Harry W. Rudel,  
Roselle Park, N. J., assignors to Standard Oil  
Development Company, a corporation of Dela-  
ware

No Drawing. Application December 14, 1946,  
Serial No. 716,432

11 Claims. (Cl. 44—69)

1

This invention relates to motor fuels and relates more particularly to the stabilization of tetraethyl lead in motor fuels.

It is common practice to add to motor fuels a fluid composition consisting principally of tetraethyl lead and small amounts of ethylene dibromide, ethylene dichloride and other substances, in order to increase the antiknock value of the motor fuel. Most of the gasoline now being sold contains some of this fluid, the amount varying from about 1-3 ccs. per gallon of gasoline. Fuel for special purposes such as aviation gasoline may contain even more.

It has been found that upon storage, and especially upon exposure to sunlight, the tetraethyl lead tends to deteriorate or decompose with the production of a haze or cloud formation in the gasoline and with subsequent deposition of a white precipitate. These lead deposits are most noticeable in sight glasses and in the glass bowls of gasoline pumps which become fouled and require frequent cleaning. Loss of the lead compound through precipitation also tends to lower the antiknock value of the motor fuel.

It has now been found that the addition of a very small amount of the product obtained by the polymerization of alpha-beta unsaturated acid esters will stabilize the lead tetraethyl and retard deposition of deteriorated or partially decomposed tetraethyl lead, and furthermore will prevent the corrosion of metals in contact with wet fuel containing lead tetraethyl.

Polymerized alpha-beta unsaturated esters which may be employed in accordance with our invention to stabilize lead tetraethyl include polymerized esters of acrylic acid, methacrylic acid, fumaric acid, maleic acid, itaconic acid and mesaconic acid and polymerized vinyl esters of fatty acids. These polymers should have a molecular weight of 2,000 to 30,000 or even higher and should be soluble in motor fuel.

The amount of stabilizer used depends on the amount of tetraethyl lead in the gasoline. It has been found that ordinarily 0.1 to 1% by weight of the above stabilizers based on the total weight of gasoline is sufficient for most purposes.

The stabilizers may be added to the gasoline directly or, if necessary, dissolved in a suitable solvent and then added to the gasoline in desired proportions.

The stabilizers may also be added to motor fuel adjuncts such as benzene or alcohol, antioxidants, solvent oils, deactivators etc., or with metal salts of acidic cyanic compounds etc. These stabilizers may be added directly to the ethyl fluid with additional amounts of solvent, if necessary, and sold and shipped in this form. In this way the addition of tetraethyl lead to gasoline and addition of stabilizer occur simulta-

neously, thus avoiding any chance of decomposition after the addition of ethyl fluid.

In order to illustrate the effectiveness of these stabilizers, a number of them were tested under conditions tending to cause the decomposition of the tetraethyl lead. In these tests a sample of commercial aviation motor fuel containing 4 cc. of lead tetraethyl in a clear glass bottle was exposed to direct sunlight. Samples of the same gasoline but containing 0.01, 0.1 and 1.0% of various stabilizers of this invention were also exposed to the direct sunlight in the same manner. The results are given in the following table.

| Polymer                                                                                                                                    | Concentration Wt. Per Cent Based on the Gasoline | Precipitation On Exposure to Sunlight |                                                  |
|--------------------------------------------------------------------------------------------------------------------------------------------|--------------------------------------------------|---------------------------------------|--------------------------------------------------|
|                                                                                                                                            |                                                  | 1 Day                                 | 7 Days                                           |
| A commercial methacrylic polymer having a molecular weight of about 15,000 prepared by Rohm and Haas.                                      | 0.01<br>0.10<br>1.0                              | trace<br>none<br>do                   | heavy.<br>Do.<br>light.                          |
| An ester formed from fumaric acid and an alcohol with 1% benzoyl peroxide for 15 hours at 80° C. having a molecular weight of about 2,000. | 0.01                                             | trace                                 | heavy.                                           |
| Copolymer of decyl maleate-vinyl acetate. <sup>1</sup>                                                                                     | 0.10<br>0.10<br>1.0                              | none<br>do<br>do                      | medium.<br>light.<br>very light.<br>none.<br>Do. |
| None                                                                                                                                       |                                                  | heavy                                 | very heavy.                                      |

<sup>1</sup> Prepared by polymerizing a mixture of 75% decyl maleate and 25% vinyl acetate with 1% benzoyl peroxide in 70% mineral oil solution for 16-24 hours at 80° C. and has a molecular weight of about 15,000.

The corrosion inhibiting action of the polymers in wet gasoline (2 cc. water added to 50 cc. of commercial aviation fuel containing 4 cc. lead) stored in contact with polished steel test strips is indicated by the following data.

| Polymer                                                                                                                                    | Conc.<br>Wt. Per<br>Cent | Corrosion of Iron Test Strip |                                     |
|--------------------------------------------------------------------------------------------------------------------------------------------|--------------------------|------------------------------|-------------------------------------|
|                                                                                                                                            |                          | 1 Day                        | 7 Days                              |
| A commercial methacrylic polymer having a molecular weight of about 15,000 prepared by Rohm and Haas.                                      | 0.10<br>1.0              | Medium<br>do                 | Heavy.<br>Do.                       |
| An ester formed from fumaric acid and an alcohol with 1% benzoyl peroxide for 15 hours at 80° C. having a molecular weight of about 2,000. | 0.10<br>1.0              | Very Light<br>do             | Medium.<br>Light.                   |
| Copolymer of decyl maleate and vinyl acetate.                                                                                              | 0.10<br>1.0              | Trace<br>None<br>Heavy       | Very Light.<br>None.<br>Very Heavy. |

55 The nature and objects of the present invention having been thus described and illustrated, what is claimed as new and useful and is desired to be secured by Letters Patent is:

1. A composition consisting essentially of tetraethyl lead and a small but stabilizing amount

of a polymerized alpha-beta unsaturated acid ester having a molecular weight of at least 2,000 to 30,000.

2. A composition consisting essentially of tetraethyl lead and a small but stabilizing amount of a copolymer of decyl maleate and vinyl acetate having a molecular weight of at least 2,000 to 30,000.

3. A composition consisting essentially of tetraethyl lead and a small but stabilizing amount of a polymerized fumaric acid ester having a molecular weight of at least 2,000 to 30,000.

4. A composition consisting essentially of gasoline, sufficient tetraethyl lead to increase the anti-knock properties of the fuel and 0.01-1.0 weight per cent based on the gasoline of polymerized ester of an alpha-beta unsaturated acid having a molecular weight of at least 2,000 to 30,000.

5. A composition consisting essentially of gasoline, sufficient tetraethyl lead to increase the anti-knock properties of the fuel and 0.01-1.0 weight per cent based on the gasoline of a copolymer of decyl maleate and vinyl acetate having a molecular weight of at least 2,000 to 30,000.

6. A composition consisting essentially of gasoline, sufficient tetraethyl lead to increase the anti-knock properties of the fuel and 0.01-1.0 weight per cent based on the gasoline of a polymerized

10

15

20

25

methacrylic acid ester having a molecular weight of at least 2,000 to 30,000.

7. A composition consisting essentially of a motor fuel of the gasoline type containing up to 4 cc. of lead tetraethyl sufficient to increase the antiknock properties of the fuel per gallon and from 0.01 to 1.0 weight percent of a polymerized ester of an alpha-beta unsaturated acid ester having a molecular weight of at least 2,000 to 30,000.

8. A gasoline-containing motor fuel containing tetraethyl lead in amounts sufficient to impart antiknock properties to said motor fuel and from 0.01 to 1.0 weight per cent of a polymerized ester of an alpha-beta unsaturated acid having a molecular weight of at least 2,000 to 30,000.

9. Gasoline containing about 4 cc. of tetraethyl lead per gallon and 0.01 to 1.0 weight per cent of a polymerized ester of an alpha-beta unsaturated acid having a molecular weight of at least 2,000 to 30,000.

10. A composition defined by claim 1 which contains a small amount of an ethylene halide.

11. A composition defined by claim 4 which contains a small amount of an ethylene halide.

JOHN G. McNAB.  
HARRY W. RUDEL.

No references cited.